

# United States Patent

Wade

[15] 3,637,516  
[45] Jan. 25, 1972

[54] **ALKALI METAL CYANOBOROHYDRIDE REDUCTIVE BLEACHING LIQUOR**

[72] Inventor: **Robert C. Wade, Ipswich, Mass.**

[73] Assignee: **Ventron Corporation, Beverly, Mass.**

[22] Filed: **Aug. 19, 1969**

[21] Appl. No.: **851,472**

[52] U.S. Cl.....**252/188, 8/107, 23/358,**  
162/80, 252/105

[51] Int. Cl.....**D21c 9/10, D06l 3/10**

[58] Field of Search.....**252/188, 105; 23/358; 8/107,**  
**8/101; 162/80, 81**

[56] **References Cited**

UNITED STATES PATENTS

2,992,885 7/1961 Jackson et al. ....**23/358**  
3,179,639 4/1965 Hutchinson.....**260/83.3**

3,318,657 5/1967 Wade.....**8/107**

*Primary Examiner*—Richard D. Lovering

*Assistant Examiner*—Irwin Gluck

*Attorney*—J. Harold Boss

[57]

## ABSTRACT

The invention provides an aqueous reductive bleaching liquor containing the material to be bleached selected from ground-wood pulp, kraft pulp, chemigroundwood pulp and clay dispersed therein in conventional amounts. As the reducing agent, a cyanoborohydride is dissolved in the liquor in an amount between about 0.01 and about 0.3 percent based upon the dry weight of the selected material to be bleached. The liquor has a pH between about 3 and 6 and is stable at a temperature between room temperature and about 180° F. The cyanoborohydride is selected from lithium, potassium, and sodium cyanoborohydride, sodium cyanoborohydride being preferred.

6 Claims, No Drawings

## ALKALI METAL CYANOBOROHYDRIDE REDUCTIVE BLEACHING LIQUOR

The invention relates to the reductive bleaching of ground-wood pulp, kraft pulp, chemigroundwood pulp, and clay.

The reductive bleaching of groundwood pulp and kraft pulp which contains —5 percent or more of residual liquor as well as clay has long been practiced. Sodium and zinc hydrosulfite have been the bleaching agents of choice. These materials have certain disadvantages, however, which cause a severe problem to pulp, paper and clay producers. The sulfur residues from the bleaching operation are acidic and cause problems of corrosion of equipment and the Fourdrinier wire. Appreciable amounts of hydrogen sulfide can be found in many pulp or paper mill waters which come from the hydrosulfite bleaching operation. Zinc hydrosulfite is generally preferred because of its greater stability than sodium hydrosulfite in the preferred bleaching pH range, namely, pH of 4 to 6. However, the latter material has the problem of contributing to stream pollution in the form of zinc ions which are known to be highly toxic to fish life.

Attempts to use the alkali metal borohydrides as reductive bleaching agents for these pulps and clay have not been successful because of the rapid hydrolysis of these borohydrides at a pH below 9. While some bleaching can be accomplished with these borohydrides, inordinately large and uneconomical amounts of these borohydrides (5 to 20 pounds per ton of dry pulp or clay) are required to accomplish the desired bleaching.

I have discovered that the above problems and difficulties can be overcome by the use of an alkali metal cyanoborohydride as the reducing agent and that small and economical amounts effectively bleach liquor-containing wood pulps, such as groundwood, chemigroundwood or kraft pulps, and clay. For reasons of economics, I prefer to use sodium cyanoborohydride ( $\text{NaBH}_3\text{CN}$ ). The conventional method and equipment used when the reducing agent is hydrosulfite is used when a cyanoborohydride is used as the reducing agent, except that a lower pH of between about 3 to 6 may be used and a smaller quantity of the cyanoborohydride is required. No corrosive residues remain after the bleaching operation is complete.

Thus the invention provides an aqueous reductive bleaching liquor containing the material to be bleached dispersed therein and an amount of cyanoborohydride dissolved therein between about 0.01 and about 0.3 percent by weight based upon the dry weight of the selected material to be bleached. This aqueous reductive bleaching liquor has a pH between about 3 and 6 and is stable at a temperature between room temperature and about 180° F.

Sodium and lithium cyanoborohydride may be economically synthesized by a process described in my copending patent application Ser. No. 833,722, filed June 16, 1969. The method comprises mixing substantially anhydrous hydrogen cyanide with substantially anhydrous lithium or sodium borohydride at a temperature between 0° C. and 100° C. in a substantially anhydrous solvent, such as tetrahydrofuran. The process for preparing potassium cyanoborohydride is described in my copending U.S. Pat. application Ser. No. 833,766, filed June 16, 1969, the process being similar to that for preparing the sodium and lithium cyanoborohydrides, except that dimethyl formamide must be used as the solvent.

The invention is illustrated further by the following specific examples.

## EXAMPLE 1

The groundwood pulp used for these experiments was a southern pine. The consistency was adjusted to 3 percent. All tests were run on 10 grams of oven dry pulp. Bleaching was

carried out in polyethylene bags in a constant temperature bath at 140° F. for 1 hour at a pH of 4.0. Then, a pulp sheet was prepared and dried by standard procedures. Brightness measurements were made on a photovolt reflectance meter.

| 5  | % $\text{NaBH}_3\text{CN}$<br>(on wt. of O.D. pulp) | Brightness | Brightness<br>Gain |
|----|-----------------------------------------------------|------------|--------------------|
| 10 | Control                                             | 61.3       | —                  |
|    | 0.25                                                | 67.0       | 5.2                |
|    | 0.095                                               | 65.8       | 4.1                |
|    | 0.031                                               | 63.9       | 2.2                |

## EXAMPLE 2

15 Kraft liner board pulp was bleached at pH = 4, 140° F. for 15 minutes. Results are summarized below:

| 20 | % $\text{NaBH}_3\text{CN}$<br>(on wt. of O.D. pulp) | Brightness | Brightness<br>Gain |
|----|-----------------------------------------------------|------------|--------------------|
| 25 | Control                                             | 18.0       | —                  |
|    | 0.25                                                | 22.8       | 4.8                |
|    | 0.09                                                | 21.0       | 3.0                |

25 There was a marked shift in color from red to yellow in these pulps.

## EXAMPLE 3

1000 g. of unbleached clay (J. M. Huber Co. "Hydrogloss") 30 was slurried in 2,000 g.  $\text{H}_2\text{O}$ . pH of the slurry was adjusted to 4.  $\text{NaBH}_3\text{CN}$  was added as a 5 percent solution in water to give the desired amount based on the weight of clay. Bleaching was carried out at room temperature for 1 hour. The clay was then vacuum filtered and dried at 100° C. in an 35 air oven. Brightness was measured on a "Photovolt" reflectance meter. Results are summarized in the following table.

| 40 | % $\text{NaBH}_3\text{CN}$<br>(based on wt. dry clay) | Brightness | Brightness<br>Gain |
|----|-------------------------------------------------------|------------|--------------------|
| 45 | Control                                               | 74.0       | —                  |
|    | 0.05                                                  | 76.0       | 2                  |
|    | 0.1                                                   | 78.0       | 4                  |
|    | 0.2                                                   | 81.5       | 7.5                |

I claim:

1. An aqueous reductive bleaching liquor comprising a material selected from the group consisting of groundwood pulp, kraft pulp, chemigroundwood pulp and finely divided 50 clay dispersed therein, said liquor having an amount of a cyanoborohydride between about 0.01 and about 0.3 percent by weight based upon the dry weight of said selected material dissolved therein and having a pH between about 3 and 6 and being stable at a temperature between room temperature and 55 about 180° F., said cyanoborohydride being selected from the group consisting of lithium, sodium, and potassium cyanoborohydrides.
2. An aqueous reductive bleaching liquor as claimed by 60 claim 1 wherein said cyanoborohydride is sodium cyanoborohydride.
3. An aqueous reductive bleaching liquor as claimed by 65 claim 2 wherein said material is groundwood pulp.
4. An aqueous reductive bleaching liquor as claimed by claim 2 wherein said material is kraft pulp.
5. An aqueous reductive bleaching liquor as claimed by 70 claim 2 wherein said material is chemigroundwood pulp.
6. An aqueous reductive bleaching liquor as claimed by claim 2 wherein said material is clay.

\* \* \* \* \*